

April 4, 1950

G. G. CHISHOLM

2,502,704

APPARATUS FOR CONCENTRATING ORES CENTRIFUGALLY

Filed Sept. 13, 1947

2 Sheets-Sheet 1



INVENTOR

G. G. CHISHOLM

By: Fetherstonhaugh & Co,  
ATT'YS

April 4, 1950

G. G. CHISHOLM

2,502,704

APPARATUS FOR CONCENTRATING ORES CENTRIFUGALLY

Filed Sept. 13, 1947

2 Sheets-Sheet 2



Fig. 4



Fig. 2



Fig. 3

INVENTOR

G. G. CHISHOLM

By: Fetherstonhaugh & Co.  
ATT'YS

## UNITED STATES PATENT OFFICE

2,502,704

APPARATUS FOR CONCENTRATING ORES  
CENTRIFUGALLY

Gilbert Gordon Chisholm, London, Ontario, Canada, assignor to Ferros Metals Research Co., Limited, Toronto, Ontario, Canada, a company of Ontario

Application September 13, 1947, Serial No. 773,887

2 Claims. (Cl. 233—27)

1

This invention generally relates to a method for separating ore pulps into a concentrate and a tailing, and to an apparatus for accomplishing the method of the invention. More particularly, the invention discloses a method and apparatus for centrifugally concentrating low grade ores in a continuous manner.

Most of the readily accessible high-grade iron-ore deposits in North America have been depleted, and the tenor of iron-ores beneficiated has been continually decreasing. Such low-grade deposits are now being worked that standard concentrating methods have been found wanting when applied to these ores, since substantial losses accompany the employment of these methods.

It is therefore an object of the present invention to beneficiate low-grade iron ores with a minimum of loss of values.

A further object of the invention is to inexpensively and efficiently concentrate low-grade iron ores.

A further object of the invention is to continuously separate various ores into a concentrate and a tailing.

A further object of the invention is to provide an apparatus of simple construction adapted to concentrate ores through centrifugal action.

A still further object of the invention is to provide a centrifugal ore concentrator which is sturdy, durable, and economical of manufacture.

With these and other objects in view, the invention generally comprises continuously separating an ore pulp into a concentrate and a tailing by leading the pulp into a plurality of open-ended tubes angularly disposed on a rotating means, rotating said tubes at high speeds, continuously removing a tailing from the ends of the tubes, and continuously removing a concentrate from an area of the inner peripheral edges of the tubes.

Other objects of the invention will be apparent from a study of the following detailed specification taken in conjunction with the accompanying drawings.

In the drawings:

Figure 1 is a vertical section of an apparatus adapted to carry out the method of my invention,

Figure 2 is an enlarged vertical section of the concentrate withdrawal means, and

Figure 3 is a plan section of the concentrate withdrawal means.

Referring particularly to Figure 1, numeral 10 represents a vertical spindle. A sleeve 11 is rotatably mounted on spindle 10 by means of thrust

2

bearings 12 and bushings 13 and 14. A drive pulley 15, adapted to receive a belt, is attached to sleeve 11, whereby the sleeve may be belt-driven. Two discs, or spiders 16 and 17 attached to sleeve 11, support a plurality of open-ended concentrating tubes 18 at an angle to the axis of spindle 10. A feed distributor head 19 is fixedly mounted on the rotatable sleeve 11 and rotates therewith. Distributing tubes 20 connect distributor head 19 with each of the concentrating tubes 18.

A cylindrical screen 21 may be mounted within each tube 18. Each tube 18 is provided with a concentrate discharge slot 22 in the wall of the tube adjacent the outer end thereof. A spigot collar 23 is concentrically mounted on said tube in the area of slot 22. A discharge spout 24 extends from spigot collar 23 and the latter is further provided with an orifice 25. A splitter 26 is disposed within tube 18 to direct the concentrate toward discharge spout 24. The positions of a splitter in the form of a deflector plate 26 and spout 24, relative to discharge slot 22, may be varied by means of a stud 27, attached to the splitter and projecting through orifices 25 in spigot collar 23. The outer end of stud 27 is threaded and is provided with a nut 28, by means of which stud 27 may be clamped to spigot collar 24. A concentrate launder 29 is arranged below concentrate discharge spouts 24, and a tailings launder 30 is disposed below the outer ends of the tubes.

Tubes 18 have been shown in the drawing as straight in form. Actually, I prefer to use curved tubes angularly disposed on sleeve 11, and I prefer to so curve the tubes that they approach the vertical at their outer ends. In this construction, concentrate discharge spout 24 extends outwardly substantially at right angles to spigot collar 23.

The method of operation is as follows. The machine is set in motion, causing the tubes 18 to revolve about the fixed spindle 10. (With low grade iron ores, I prefer to use speeds somewhat in excess of 1000 revolutions per minute. Considerably greater or lesser speeds are employed, however, with other ores.) Comminuted ore, in the form of a liquid pulp, is fed into the distributor head 19, and is thrown by centrifugal force 50 to the sides of the latter, and thence through distributor tubes 20 to concentrating tubes 18. As the pulp passes down the tubes 18 under the influences of gravity and of centrifugal force, particles of relatively high specific gravity tend to 55 concentrate along the inner walls of tubes 18.

over an area the direction of travel of the tubes, and particles of lesser specific gravity are forced toward the inner part of the tube, replacing the higher gravity particles. (When the machine is rotating at slow speeds, some surface tension exists between the liquid-solid interfaces of the liquid and the ore particles. Such surface tension is eliminated by the passage of the particles through the screen 21.) As the pulp approaches the outer ends of the tubes, the concentrating, or sorting through specific gravity differences, is completed. If a horizontal section is taken through the pulp mass at this time, the mass will be found to be in the form of a segment of a circle, the chord of said segment being substantially radially disposed with regard to said spindle; and if an analysis were made of the values of material constituting this segmental form, it would be found that the values were concentrated over the area of the segment remote from the spindle whereas the area nearest the spindle was substantially deplete of values. The downward travel of the pulp mass is interrupted by the splitter 26 which directs the enriched portion of the pulp to concentrate discharge slot 22, whence it is thrown through concentrate discharge spout 24 into concentrate launder 29. The depleted portion of the pulp passes by the splitter, and is thrown out of the ends of the tubes into tailings launder 30. The tailings may be dumped, or may be repassed through the same concentrator, or a similar one, in order to further clean the tailings.

Modifications of the method and of the apparatus will be apparent to persons of mechanical ability and persons familiar with the dressing of ores. It is therefore intended that the present disclosure should not be limited in any way other than that indicated by the scope of the following claims.

What I claim as my invention is:

1. Apparatus for continuously dressing an ore pulp into a concentrate and a tailing, comprising

5 ing, a substantially vertical rotatable member, at least one tubular member mounted at an acute angle on said rotatable member and having an inner open end and an outer open end, means for feeding an ore pulp into the inner open end of said tubular member, a splitter in the form of a deflector plate mounted within said tubular member near its outer end, and extending only partially across the interior of said tubular member to allow passage of tailing and discharge of the same from the outer end of said tubular member, a discharge opening formed in the wall of said tubular member adjacent said deflector plate to accommodate concentrate deflected by 10 said plate exteriorly of said tubular member, an adjustable spigot collar in the form of a sleeve-like member slidably mounted on said tubular member and having a discharge opening and a spout mounted thereon about the opening designed to register with the discharge opening in 15 said tubular member, and means passing through said discharge opening for connecting said spigot collar to said deflector plate.

2. Apparatus as claimed in claim 1, in which the discharge opening extends circumferentially of the tubular member a radial dimension of substantially 180 degrees.

GILBERT GORDON CHISHOLM.

#### REFERENCES CITED

30 The following references are of record in the file of this patent:

#### UNITED STATES PATENTS

| 35 | Number    | Name       | Date           |
|----|-----------|------------|----------------|
|    | 730,114   | Guttner    | June 2, 1903   |
|    | 935,311   | Raist      | Sept. 28, 1909 |
|    | 943,083   | Kuchs      | Dec. 14, 1909  |
| 40 | 1,014,827 | King       | Jan. 16, 1912  |
|    | 1,014,849 | Richardson | Jan. 16, 1912  |
|    | 1,111,600 | Mauss      | Sept. 22, 1914 |
|    | 1,139,206 | McGovern   | May 11, 1915   |
|    | 2,185,279 | Strezynski | Jan. 2, 1940   |